

## UNITED STATES PATENT OFFICE

WILLIAM J. WOOLDRIDGE, OF MANSFIELD, OHIO

## PROCESS FOR THE MANUFACTURE OF SILICON STEEL

No Drawing.

Application filed May 26, 1928. Serial No. 280,953.

This invention relates to a process for the manufacture of silicon-steel in the form of plates and sheets adapted for use in electrical apparatus, such as reactors, transformers, 5 and the like.

The invention has for its object generally the provision of an improved process for producing plates and sheets of the character specified, which have better mechanical and 10 electrical properties than those heretofore manufactured, in a manner which is both efficient and economical.

More particularly, an object of the invention is to reduce substantially to a minimum 15 the scale which forms on silicon-steel in the process of its manufacture, and at the same time to provide silicon-steel sheets or plates which have the properties of a well-annealed steel.

20 Other objects of the invention will in part be obvious and will in part appear herein-after.

The invention accordingly comprises the 25 several steps and the relation and order of one or more of such steps with respect to each of the others thereof, which will be exemplified in the process hereinafter disclosed, and the scope of the application of which will 30 be indicated in the claim.

35 Steel which has been rolled and given heat treatments is known to develop a film of oxides or scale over its surface. This scale is brittle and prevents the steel laminations or punchings from being manufactured with desired facility.

To eliminate the undesirable effects of scale, pickling the plates and sheets has been proposed. This pickling removes the scale 40 and, as a rule, improves the surface appearance of the plates and sheets. After the pickling the sheets may again be rolled if desired.

In producing sheets and plates of silicon-45 steel for electrical apparatus it is not the surface appearance that it is desired to improve by pickling, as this is of secondary consideration. I have ascertained, in order to improve the electrical qualities that all the 50 rolling should be done before the pickling

stage, and in order that the sheets and plates have desired magnetic properties, viz, low core losses and high permeability, they should be annealed again after the pickling.

In brief, in accordance with the present 55 invention, the plates or sheets of silicon-steel are first hot-rolled, and then cold-rolled, after which they are annealed at the usual temperature for such material. After the sheets or plates have become cold, they are 60 then pickled and dried, and then re-annealed at a comparatively low temperature. When this cycle of operations is completed, the sheets and plates are ready for use.

At the beginning of the cycle, heated plates 65 or ingots are hot-rolled in any suitable mill, until they have been reduced in thickness to a gauge roughly approximating the desired gauge, for example, to within a few per cent. of the desired final gauge. When the hot rolling has been completed, the plates are allowed to cool, and then are cold-rolled in a finishing mill until the desired gauge is attained. When this rolling is completed, 70 the grain is fully developed.

75 After the plates or sheets have thus been fully rolled, they may be comparatively hard and brittle. In the next step of the process the sheets or plates are given their first anneal. This is accomplished by heating the 80 sheets and plates when placed in suitable groups or stacks in the heating chamber of any suitable furnace, for example, a muffle furnace which is heated substantially to the usual temperatures employed for silicon-steel sheets, i. e., to a temperature of about 700 to 800 degrees C. Such temperature is held for a proper period, for example, 4 to 8 85 hours, after which the furnace is permitted to cool and the sheets removed.

90 After the first anneal, the sheets or plates are then pickled by placing them in vats where they are subjected to a bath of highly dilute acid, for example, a solution containing 5 per cent. of hydrochloric or sulphuric acid. During the annealing step the sheets in the annealing furnace have considerable scale 95 formed on their surfaces which appears as a brittle incrustation entirely enveloping the 100

sheet. Such scale contains a relatively high percentage of silicon oxide, ( $SiO_2$ ), and as a result is very hard and readily cracks. While the inner core of a silicon-steel sheet has been made pliant and malleable by the anneal, the sheet, as a whole, is by no means in a desirable condition for working in punch presses and the like until the scale has been properly removed, this being accomplished in the pickling bath.

When properly pickled, the plates or sheets are taken from the pickling bath and are dried by subjecting them to a draft of relatively dry air. This air is preferably slightly warmed in order to hasten the drying step.

When pickled and dried, the sheets are given their second anneal. In order to accomplish this second annealing step, the sheets are placed for a second time in an annealing furnace where they are heated to a comparatively low temperature for silicon-steel anneals. This temperature may be, for example, 300 degrees C. This second anneal may be effected by placing the sheets or plates in the oven of a muffle furnace in suitable stacks and bringing them gradually up to the desired temperature, and holding the same at such temperature for about 4 hours, after which the heat is shut off and the sheets allowed gradually to cool before they are brought again into the outer atmosphere.

By the process of the present invention the re-annealed silicon-steel sheets or plates possess desired electrical and mechanical properties in relatively high degrees.

The cold-rolling, prior to the first anneal practiced as above described, provides for the development of a definite grain in the metal without ingrainning into the metal any substantial amount of refractory material, such as the scale which has heretofore at times been rolled into the metal. Silicon-steel sheets which contain this material have a high degree of attrition, and, as a result, quickly wear out the edges of dies and other tools designed for working and cutting the same into stampings.

By the process of the present invention silicon-steel sheets and plates are produced which are substantially free from scale, have a clear surface, possess a high degree of malleability, and can be cut in punch presses with relatively little wear on the dies. The dies of steel which are employed in such instances have substantially three times the life which they would have had cutting ordinary silicon-steel sheets and plates. Moreover, the grain of the metal initially developed is not lost during the annealing steps practiced as herein taught. As a result the silicon-steel sheets and plates produced by the present process have relatively high electrical permeabilities and show relatively low hysteresis losses even when working up to flux densities as high as 17,000 gauss or lines per square centimeter.

Silicon-steel plates and sheets, which have substantially the following composition by analysis:

|            | Per cent       |    |
|------------|----------------|----|
| Iron       | 99.00 to 95.00 | 70 |
| Silicon    | 0.5 to 4.50    |    |
| Carbon     | 0.1 to .10     |    |
| Manganese  | Approx. .12    |    |
| Sulphur    | Approx. .03    |    |
| Phosphorus | Approx. .02    | 75 |

show, when tested for hysteresis losses in an Epstein testing apparatus, losses of from 0.5 to 3.00 watts per pound at a frequency of 60 cycles and a flux density of 10,000 lines per square centimeter, depending upon the thickness of plate or sheet as well as on the analysis.

Since certain changes may be made in carrying out the above process without departing from the scope of the invention, it is intended that all matter contained in the above description shall be interpreted as illustrative and not in a limiting sense.

Having described my invention, what I claim as new and desire to secure by Letters Patent is:

The process of manufacturing silicon-steel sheets and plates, which comprises hot-rolling said sheets in a standard mill until within a few per cent. of their desired gauge, cold-rolling the same in a finishing mill until the desired gauge is attained, annealing the same at usual temperature for such material, pickling and drying the same, and thereafter re-annealing the same at a temperature not substantially greater at any time than 300 degrees C.

In testimony whereof I affix my signature.

WILLIAM J. WOOLDRIDGE.

105

110

115

120

125

130

**CERTIFICATE OF CORRECTION.**

**Patent No. 1,773,157.**

**Granted August 19, 1930, to**

**WILLIAM J. WOOLDRIDGE.**

**It is hereby certified that error appears in the printed specification of the above numbered patent requiring correction as follows: Page 2, line 72, in the table, for carbon "0.1 to .10" read .01 to .10; and that the said Letters Patent should be read with this correction therein that the same may conform to the record of the case in the Patent Office.**

**Signed and sealed this 21st day of October, A. D. 1930.**

**M. J. Moore,  
Acting Commissioner of Patents.**

**(Seal)**